



US011763980B2

(12) **United States Patent**  
**Sakai**

(10) **Patent No.:** US 11,763,980 B2  
(45) **Date of Patent:** Sep. 19, 2023

(54) **COIL COMPONENT**

(71) Applicant: **Murata Manufacturing Co., Ltd.**,  
Kyoto-fu (JP)

(72) Inventor: **Takashi Sakai**, Nagaokakyo (JP)

(73) Assignee: **Murata Manufacturing Co., Ltd.**,  
Kyoto-fu (JP)

(\*) Notice: Subject to any disclaimer, the term of this  
patent is extended or adjusted under 35  
U.S.C. 154(b) by 456 days.

(21) Appl. No.: **16/985,204**

(22) Filed: **Aug. 4, 2020**

(65) **Prior Publication Data**

US 2021/0043360 A1 Feb. 11, 2021

(30) **Foreign Application Priority Data**

Aug. 5, 2019 (JP) ..... 2019-143746

(51) **Int. Cl.**

**H01F 27/28** (2006.01)  
**H01F 27/24** (2006.01)  
**H01F 41/04** (2006.01)  
**H01F 27/29** (2006.01)

(52) **U.S. Cl.**

CPC ..... **H01F 27/2804** (2013.01); **H01F 27/24**  
(2013.01); **H01F 27/29** (2013.01); **H01F**  
**41/043** (2013.01); **H01F 2027/2809** (2013.01)

(58) **Field of Classification Search**

CPC ..... H01F 27/28  
See application file for complete search history.

(56) **References Cited**

**U.S. PATENT DOCUMENTS**

2003/0134612 A1 7/2003 Nakayama et al.  
2011/0037557 A1\* 2/2011 Konoue ..... H01F 27/34  
336/200

**FOREIGN PATENT DOCUMENTS**

|    |               |   |         |       |              |
|----|---------------|---|---------|-------|--------------|
| CN | 110033930 A   | * | 7/2019  | ..... | H01F 17/0013 |
| JP | 2002043156 A  |   | 2/2002  |       |              |
| JP | 2009-302580 A |   | 12/2009 |       |              |
| JP | 2009302580 A  | * | 12/2009 | ..... | H01F 17/0013 |
| JP | 2010-040860 A |   | 2/2010  |       |              |
| JP | 2010040860 A  | * | 2/2010  |       |              |
| JP | 2012-195471 A |   | 10/2012 |       |              |
| JP | 2012195471 A  | * | 10/2012 |       |              |

**OTHER PUBLICATIONS**

An Office Action; "Notice of Reasons for Refusal," mailed by the  
Japanese Patent Office dated Apr. 5, 2022, which corresponds to  
Japanese Patent Application No. 2019-143746 and is related to U.S.  
Appl. No. 16/985,204 with English language translation.

\* cited by examiner

*Primary Examiner* — Marlon T Fletcher

*Assistant Examiner* — Matthew T Sarles

(74) *Attorney, Agent, or Firm* — Studebaker & Brackett  
PC

(57) **ABSTRACT**

A coil component in which a crack is rarely generated around a coil conductor layer. The coil component includes an element body; and a coil provided in the element body and spirally wound along a first direction. The coil has a plurality of coil conductor layers stacked along the first direction. The element body has a vicinity area located in a vicinity of each of the coil conductor layers, and has a non-vicinity area other than the vicinity area. The vicinity area has a pore area rate less than a pore area rate in at least a part of the non-vicinity area.

**20 Claims, 7 Drawing Sheets**



FIG. 1





FIG. 2

FIG. 3



FIG. 4



FIG. 5A



FIG. 5B



FIG. 5C



FIG. 5D



FIG. 5E



FIG. 6A



FIG. 6B



FIG. 7





FIG. 8

# 1

## COIL COMPONENT

### CROSS-REFERENCE TO RELATED APPLICATION

This application claims benefit of priority to Japanese Patent Application No. 2019-143746, filed Aug. 5, 2019, the entire content of which is incorporated herein by reference.

### BACKGROUND

#### Technical Field

The present disclosure relates to a coil component.

#### Background Art

Conventionally, examples of a coil component include one described in Japanese Patent Application Laid-Open No. 2002-043156. This coil component includes an element body and a coil in the element body. The element body includes a plurality of insulating layers that are stacked, and the coil includes a plurality of coil conductor layers that are stacked.

### SUMMARY

However, it has been found that in the conventional coil component, there is a possibility that a crack will be generated around the coil conductor layer. As a result, there is a possibility that the coil conductor layer will not be sufficiently sealed, and the reliability will be reduced.

Accordingly, the present disclosure provides a coil component in which a crack is rarely generated around a coil conductor layer.

The coil component according to the present disclosure includes an element body; and a coil provided in the element body and spirally wound along a first direction. The coil has a plurality of coil conductor layers stacked along the first direction. The element body has a vicinity area located in a vicinity of each of the coil conductor layers, and has a non-vicinity area other than the vicinity area. Also, the vicinity area having a pore area rate less than a pore area rate in at least a part of the non-vicinity area.

Here, the term "vicinity area" means an area that is located in the vicinity of the coil conductor layer and is present within 20  $\mu\text{m}$  from the surface of the coil conductor layer in the element body.

Here, the term "pore area rate" means the rate of the area of pores per unit area in a predetermined range in a section of an element body 10 along the first direction.

According to the coil component of the present disclosure, because the pore area rate in the vicinity area is less than the pore area rate in at least a part of the non-vicinity area, the vicinity area of the coil conductor layer can have reduced pores, can be dense, and has increased strength, so that the generation of a crack can be prevented.

Furthermore, in one embodiment of the coil component, the element body has a first magnetic layer and a second magnetic layer, the first magnetic layer and the second magnetic layer are alternately stacked along the first direction, and the second magnetic layer is provided on the first magnetic layer in the same layer as each of the coil conductor layers.

According to the above-described embodiment, because the second magnetic layer and the coil conductor layer are the same layer, the thickness of the coil conductor layer can

# 2

be kept, and the DC resistance value (Rdc) of the coil conductor layer can be reduced.

Furthermore, in one embodiment of the coil component, the pore area rate in the vicinity area is 1% or less.

According to the above-described embodiment, because the vicinity area is dense, the generation of a crack in the vicinity area can be prevented.

Furthermore, in one embodiment of the coil component, the pore area rate in at least a part of the non-vicinity area is 2% or more and 8% or less (i.e., from 2% to 8%).

According to the above-described embodiment, even when heat or external stress is applied to the element body, the internal stress can be further relaxed by the pores.

Furthermore, in one embodiment of the coil component, a difference between the pore area rate in the vicinity area and the pore area rate in at least a part of the non-vicinity area is 1% or more.

According to the above-described embodiment, because the vicinity area has reduced pores and is dense, the generation of a crack can be prevented, and the internal stress can be relaxed by the pores present in the non-vicinity area.

Furthermore, in one embodiment of the coil component, the element body further includes a void, the void is located between the coil conductor layers adjacent to each other along the first direction, and is in contact with one coil conductor layer of the coil conductor layers adjacent to each other.

According to the above-described embodiment, the stress on the element body can be suppressed. The stress is caused by the difference between the thermal expansion coefficients of the coil conductor layer and the element body, and is due to the change in the temperature of the coil conductor layer.

According to the present disclosure, the coil component is provided in which a crack is rarely generated around the coil conductor layer.

### 35 BRIEF DESCRIPTION OF THE DRAWINGS

FIG. 1 is a perspective view showing a first embodiment of a coil component;

FIG. 2 is a sectional view taken along the line X-X of the coil component in FIG. 1;

FIG. 3 is an exploded plan view of a coil component;

FIG. 4 is an enlarged sectional view around the coil conductor layer in FIG. 2;

FIG. 5A is an explanatory view illustrating an example of a method for manufacturing a coil component;

FIG. 5B is an explanatory view illustrating an example of the method for manufacturing a coil component;

FIG. 5C is an explanatory view illustrating an example of the method for manufacturing a coil component;

FIG. 5D is an explanatory view illustrating an example of the method for manufacturing a coil component;

FIG. 5E is an explanatory view illustrating an example of the method for manufacturing a coil component;

FIG. 6A is an explanatory view illustrating an example of a method for manufacturing a coil component;

FIG. 6B is an explanatory view illustrating an example of the method for manufacturing a coil component;

FIG. 7 is an enlarged sectional view of a coil component in a second embodiment in the vicinity of a coil conductor layer; and

FIG. 8 is a partial view of FIG. 4 illustrating the pore area rate in the vicinity area and non-vicinity area.

### DETAILED DESCRIPTION

Hereinafter, a coil component that is one aspect of the present disclosure will be described in detail with reference

to the embodiments shown in the drawings. Note that the drawings include some schematic ones and sometimes do not reflect actual dimensions or ratios.

### First Embodiment

FIG. 1 is a perspective view showing a first embodiment of the coil component. FIG. 2 is a sectional view taken along the line X-X of the first embodiment shown in FIG. 1, and is a sectional view in the LT plane passing through the center along the W axis. FIG. 3 is an exploded plan view of the coil component, and shows views from the bottom view to the top view along the T axis. The L axis is in the length direction of a coil component 1, the W axis is in the width direction of the coil component 1, and the T axis is in the height direction of the coil component 1 (the first direction).

As shown in FIG. 1, the coil component 1 has an element body 10, a coil 20 provided inside the element body 10, and a first external electrode 31 and a second external electrode 32 that are provided on the surface of the element body 10 and electrically connected to the coil 20.

The coil component 1 is electrically connected to the wire of a circuit board (not shown) via the first external electrode 31 and the second external electrode 32. The coil component 1 is used, for example, as a noise removal filter, and is used in electronic devices such as personal computers, DVD players, digital cameras, TVs, mobile phones, and car electronics.

The element body 10 is formed into a substantially rectangular parallelepiped shape. The surface of the element body 10 has a first end face 15, a second end face 16 located on the side opposite from the first end face 15, and four sides 17 located between the first end face 15 and the second end face 16. The first end face 15 and the second end face 16 face each other along the L axis.

As shown in FIG. 2, the element body 10 includes a plurality of first magnetic layers 11 and second magnetic layers 12. The first magnetic layer 11 and the second magnetic layer 12 are alternately stacked along the T axis. The first magnetic layer 11 and the second magnetic layer 12 include a magnetic material such as a Ni—Cu—Zn-based ferrite material. The first magnetic layer 11 and the second magnetic layer 12 each have a thickness of, for example, 5  $\mu\text{m}$  or more and 30  $\mu\text{m}$  or less (i.e., from 5  $\mu\text{m}$  to 30  $\mu\text{m}$ ). The element body 10 may include a nonmagnetic layer in part.

The first external electrode 31 covers the entire surface of the first end face 15 of the element body 10 and the ends of the sides 17 of the element body 10 on the first end face 15 side. The second external electrode 32 covers the entire surface of the second end face 16 of the element body 10 and the ends of the sides 17 of the element body 10 on the second end face 16 side. The first external electrode 31 is electrically connected to a first end of the coil 20, and the second external electrode 32 is electrically connected to a second end of the coil 20.

The first external electrode 31 may have an L-shape formed over the first end face 15 and one side 17, and the second external electrode 32 may have an L-shape formed over the second end face 16 and one side 17.

As shown in FIGS. 2 and 3, the coil 20 is spirally wound along the T axis. The coil 20 includes a conductive material such as Ag or Cu. The coil 20 has a plurality of coil conductor layers 21 and a plurality of extended conductor layers 61 and 62.

The two first extended conductor layers 61, the plurality of coil conductor layers 21, and the two second extended

conductor layers 62 are placed in order along the T axis and electrically connected in order via a via conductor. The plurality of coil conductor layers 21 are connected in order along the T axis to form a spiral along the T axis. The first extended conductor layer 61 is exposed from the first end face 15 of the element body 10 and connected to the first external electrode 31, and the second extended conductor layer 62 is exposed from the second end face 16 of the element body 10 and connected to the second external electrode 32. The number of the first extended conductor layers 61 and the number of the second extended conductor layers 62 are not particularly limited, and may be, for example, one.

The coil conductor layer 21 is provided on the first magnetic layer 11 in the same layer as the second magnetic layer 12. With such a configuration, the thickness of the coil conductor layer 21 can be kept, and the DC resistance value (Rdc) of the coil conductor layer 21 can be reduced. That is, the cross-section of the coil conductor layer 21 can have a rectangle shape such as a trapezoid shape. Note that in FIG. 3, the second magnetic layer 12 is omitted.

The coil conductor layer 21 is formed into a shape wound on a plane with less than one turn. The extended conductor layers 61 and 62 are formed into a linear shape. The coil conductor layer 21 has a thickness of, for example, 10  $\mu\text{m}$  or more and 40  $\mu\text{m}$  or less (i.e., from 10  $\mu\text{m}$  to 40  $\mu\text{m}$ ). The first extended conductor layer 61 and the second extended conductor layer 62 have a thickness of, for example, 10  $\mu\text{m}$  or more and 30  $\mu\text{m}$  or less (i.e., from 10  $\mu\text{m}$  to 30  $\mu\text{m}$ ), and the thickness may be less than that of the coil conductor layer 21.

In the element body 10, a void 51 may be present. The void 51 is located between the coil conductor layer 21 and the first magnetic layer 11. The void 51 is provided so as to be in contact with the lower face of the coil conductor layer 21. The void 51 is provided along the entire surface of the interface between the coil conductor layer 21 and the first magnetic layer 11, and may be provided along a part of the interface. The maximum thickness of the void 51 is, for example, 0.5  $\mu\text{m}$  or more and 8  $\mu\text{m}$  or less (i.e., from 0.5  $\mu\text{m}$  to 8  $\mu\text{m}$ ).

The void 51 may be located between the coil conductor layer 21 and the second magnetic layer 12.

By providing the void 51, the stress on the element body can be suppressed. The stress is caused by the difference between the thermal expansion coefficients of the coil conductor layer 21 and the magnetic layers 11 and 12, and is due to the change in the temperature of the coil conductor layer 21. As a result, the deterioration of the inductance and the impedance characteristics due to the internal stress can be eliminated. As described below, in the coil component according to the present disclosure, because the pore area rate in the first area is small, the electrical insulation between the coil conductor layers is ensured even when the void is provided.

FIG. 4 is an enlarged sectional view around the coil conductor layer 21 in FIG. 2. FIG. 4 shows a section in the width direction of the coil conductor layer 21, in other words, a section orthogonal to the extending direction of the coil conductor layer 21.

As shown in FIG. 4, the element body 10 has a vicinity area E and a non-vicinity area F other than the vicinity area.

Here, the vicinity area E is present within 20  $\mu\text{m}$  from the surface of the coil conductor layer 21 in the element body 10, and when the void 51 is present in contact with the coil conductor layer 21, the vicinity area E is present within 20

μm from the boundary surface between the void 51 and the magnetic layer included in the element body 10.

In FIG. 4, an alternate long and short dash line is provided so as to surround the coil conductor layer 21 and the void 51. The area surrounded by the alternate long and short dash line in the element body 10 is an example of the vicinity area E.

The pore area rate in the vicinity area E is less than the pore area rate in at least a part of the non-vicinity area F. FIG. 8 is a partial view of FIG. 4 illustrating the pore area rate in the vicinity area E and non-vicinity area F. The rate of the area of pores 53 per unit area in the vicinity area E is less than the rate of the area of pores 53 per unit area in at least a part of the non-vicinity area F, as shown in FIG. 8.

Here, the term “pore area rate” means the rate of the area of pores per unit area in a predetermined range in a section of the element body 10. Specifically, the section used for measuring the pore area rate is an LT plane in the coil component 1 and a plane passing through the center of the coil component 1 along the W axis. The center includes not only the perfect center but also the almost center.

The pore area rate is measured as described below. The section that is an LT plane in the coil component 1 and a plane passing through the center of the coil component 1 along the W axis is subjected to focused ion beam processing (FIB processing). The FIB processing is performed by vertically standing the sample to be measured and, if necessary, solidifying the periphery of the sample with a resin. The section that is an LT plane to be measured can be prepared by polishing the sample with a polishing machine along the W axis of the sample to a depth at which a substantially central portion along the W axis is exposed. Here, the FIB processing is performed using an FIB processing device SMI3050R manufactured by SII Nano Technology Inc. Then, a scanning electron microscope (SEM) photograph is taken of the prepared section. The obtained SEM photograph is analyzed using image analysis software to determine the pore area rate. As the image analysis software, “A-zo kun” (registered trademark) manufactured by Asahi Kasei Engineering Corporation is used.

In the coil component according to the present disclosure, because the pore area rate in the vicinity area E is less than the pore area rate in at least a part of the non-vicinity area F, the vicinity area E of the coil conductor layer 21 can have reduced pores, can be dense, and has increased strength, so that the generation of a crack can be prevented. There is a possibility that the crack as described above will be generated when a thermal shock is applied, for example, during reflow, or when a mechanical stress is applied.

Because the pore area rate is small in the vicinity area E, pores that serve as a current path can be reduced between the coil conductor layers 21 adjacent to each other along the first direction, and the electrical insulation between the coil conductor layers 21 adjacent to each other can be enhanced. In particular, even when the thickness of the element body 10 present between the coil conductor layers 21 adjacent to each other along the first direction is thin, the insulation between the coil conductor layers 21 adjacent to each other along the first direction can be maintained. The leak can be suppressed not only from the opposing faces of the coil conductor layers 21 adjacent to each other, but also from the side of the coil conductor layers 21.

The pore area rate in the vicinity area E is, for example, 1% or less, and specifically, 0.5% or less.

Because the vicinity area E has the pore area rate as described above, the vicinity area is dense, so that the generation of a crack in the vicinity area E can be prevented.

The pore area rate in at least a part of the non-vicinity area F is, for example, 1% or more, or 1.5% or more, and preferably 2% or more and 8% or less (i.e., from 2% to 8%).

As a result, even when heat or external stress is applied to the element body, the internal stress can be relaxed by the pores. Furthermore, the heat generated from the coil can be further dissipated by the pores. Even when the pore area rate in the non-vicinity area F is the above-described value, the generation of a crack in the vicinity area E can be prevented because the vicinity area E is dense.

The difference between the pore area rate in the vicinity area E and the pore area rate in at least a part of the non-vicinity area F is, for example, 1% or more, and specifically 2% or more.

As a result, because the vicinity area E has reduced pores and is dense, the generation of a crack can be prevented, and the internal stress can be relaxed by the pores present in the non-vicinity area F.

The size of the pore is not particularly limited, and is, for example, 0.7 μm or less, and specifically 0.6 μm or less. The lower limit of the size of the pore is, for example, 0.05 μm.

The shape of the pore is not particularly limited, and the section can substantially have, for example, a circular shape, an elliptical shape, a polygonal shape, or the like.

In another aspect, the element body 10 has a first area Z1 and a second area Z2. The first area Z1 shows an area between the coil conductor layers 21 adjacent to each other along the T axis in the element body 10. FIG. 4 shows an example of the first area Z1 as an area surrounded by an alternate long and short dash line between the opposing faces of the coil conductor layers 21 adjacent to each other. The second area Z2 shows an area other than the first area Z1 in the element body 10.

The pore area rate in the first area Z1 is less than the pore area rate in at least a part of the second area Z2.

Because the pore area rate in the first area Z1 is small, pores that serve as a current path can be reduced between the coil conductor layers 21 adjacent to each other along the T axis, and the insulation between the coil conductor layers 40 adjacent to each other can be enhanced. In particular, even when the thickness of the element body present between the coil conductor layers 21 adjacent to each other along the T axis (that is, the magnetic layer) is thin, the insulation between the coil conductor layers 21 adjacent to each other along the T axis can be maintained.

The pore area rate in the first area Z1 is, for example, 1% or less, and specifically, 0.5% or less. As a result, the pores that serve as a current path can be further reduced between the coil conductor layers 21 adjacent to each other, and the insulation between the coil conductor layers 21 adjacent to each other can be further enhanced. In particular, even when the thickness of the layer present between the coil conductor layers 21 is thin, the insulation between the coil conductor layers 21 adjacent to each other can be further maintained.

Note that only the vicinity area E may be present, or the vicinity area E and an area other than the vicinity area E may be present between the opposing faces of the coil conductor layers adjacent to each other. In other words, the entire first area Z1 may be included in the vicinity area E, or the first area Z1 may include an area that is not included in the vicinity area E.

The pore area rate in the second area Z2 is, for example, 1% or more, or 1.5% or more, and specifically 2% or more and 8% or less (i.e., from 2% to 8%).

Even when the pore area rate in the second area Z2 is a value as described above, the insulation in the coil component according to the present disclosure can be maintained.

without any problem. Furthermore, because the pore area rate in the second area Z2 is a value as described above, the internal stress can be relaxed by the pores even when heat or an external stress is applied to the element body 10.

The difference between the pore area rate in the first area Z1 and the pore area rate in at least a part of the second area Z2 is, for example, 1% or more, and specifically 2% or more.

As a result, the electrical insulation between the coil conductor layers 21 can be further enhanced, and the internal stress can be relaxed by the pores even when heat or external stress is applied to the element body 10.

In another aspect, the second area Z2 includes an out-of-vicinity area that is other than the first area Z1 and is located outside the vicinity area E. The pore area rate in the first area Z1 is less than the pore area rate in the out-of-vicinity area, and the pore area rate in the vicinity area E is less than the pore area rate in the out-of-vicinity area.

As a result, the leak generated between the coil conductor layers 21 can be further suppressed. In particular, the leak can be suppressed not only from the opposing faces of the coil conductor layers adjacent to each other, but also from the side of the coil.

In one aspect, the second area Z2 can include a central area that is in an area within a predetermined range from the central axis of the coil in the element body 10. The pore area rate in the vicinity area E is preferably less than the pore area rate in the central area. Here, the term "central area" means an area within 10  $\mu\text{m}$  from the central axis of the coil when viewed along the T axis of the coil.

With such a configuration, even when heat or external stress is applied to the element body, the internal stress can be relaxed by the pores because there are many pores in the central area.

The pore area rate in the central area is, for example, 1.0% or more, or 1.5% or more, and specifically 2% or more and 8% or less (i.e., from 2% to 8%).

Next, an example of a method for manufacturing the coil component 1 will be described with reference to FIGS. 5A to 5E and 6A to 6B.

FIGS. 5A to 5E show a section in the width direction of the coil conductor layer 21, in other words, a section orthogonal to the extending direction of the coil conductor layer 21.

First, a first magnetic sheet 211 included in the first magnetic layer 11 is provided. The first magnetic sheet 211 can be prepared by, for example, molding a magnetic slurry containing a magnetic ferrite material 111 into a sheet shape and, if necessary, processing the sheet-shaped slurry by punching or the like. In addition, a predetermined portion in the first magnetic sheet 211 is irradiated with a laser to form a through hole.

Examples of the method for processing the magnetic slurry into a sheet shape include a doctor blade method. The obtained sheet has a thickness of, for example, 15  $\mu\text{m}$  or more and 25  $\mu\text{m}$  or less (i.e., from 15  $\mu\text{m}$  to 25  $\mu\text{m}$ ).

The composition of the magnetic ferrite material 111 is not particularly limited, and, for example, a material containing  $\text{Fe}_2\text{O}_3$ ,  $\text{ZnO}$ ,  $\text{CuO}$ , and  $\text{NiO}$  can be used. When the magnetic ferrite material 111 contains  $\text{Fe}_2\text{O}_3$ ,  $\text{ZnO}$ ,  $\text{CuO}$ , and  $\text{NiO}$ , the content of  $\text{Fe}_2\text{O}_3$  is, for example, in the range of 40.0 mol % or more and 49.5 mol % or less (i.e., from 40.0 mol % to 49.5 mol %), the content of  $\text{ZnO}$  is, for example, in the range of 5 mol % or more and 35 mol % or less (i.e., from 5 mol % to 35 mol %), the content of  $\text{CuO}$  is, for example, in the range of 8 mol % or more and 12 mol % or less (i.e., from 8 mol % to 12 mol %), and the content of  $\text{NiO}$  is, for example, in the range of 8 mol % or more and

40 mol % or less (i.e., from 8 mol % to 40 mol %). The magnetic ferrite material 111 can further contain an additive. Examples of the additive include  $\text{Mn}_3\text{O}_4$ ,  $\text{Co}_3\text{O}_4$ ,  $\text{SnO}_2$ ,  $\text{Bi}_2\text{O}_3$ , and  $\text{SiO}_2$ .

5 The magnetic ferrite material 111 is wet-mixed and wet-ground by an ordinary method, and then dried. The resulting dried product is calcined at 700°C. or more and less than 800°C. (i.e., from 700°C. to 800°C.), specifically 700°C. or more and 720°C. or less (i.e., from 700°C. to 720°C.) to form a raw material powder 112. Note that there is a possibility that the raw material powder (calcined powder) 112 will contain an inevitable impurity.

An aqueous acrylic binder and a dispersant are added to the raw material powder 112, and the mixture is wet-mixed and wet-ground to prepare a magnetic slurry. The wet-mixing and wet-grinding can be performed by, for example, putting in a pot mill together with a partially stabilized zirconia (PSZ) ball.

15 On the first magnetic sheet 211, for example, a resin material is screen-printed to form a burned-out portion 41. The burned-out portion 41 is a portion that is to be burned out by firing, and the burned-out portion 41 is burned out to form the void 51 in the coil component 1 at the firing process. As the resin material, a paste material containing a resin and a solvent can be used. Examples of the resin include a resin that is burned out during firing, such as an acrylic resin. Examples of the solvent include a solvent that is burned out during firing, such as isophorone.

20 A coil conductor composition 221 included in the coil conductor layer 21 is provided by, for example, screen-printing so that the coil conductor composition 221 and the burned-out portion 41 are stacked. The coil conductor composition 221 may be, for example, a paste, and specifically, a paste containing an Ag powder, a solvent, a resin, and a dispersant can be used. Examples of the solvent include eugenol, and examples of the resin include an ethyl cellulose. In preparing the above-described paste conductor composition, an ordinary method can be used. For example, the paste conductor composition can be prepared by mixing the 25 Ag powder, the solvent, the resin, and the dispersant with a planetary mixer, and then dispersing the mixture with a three-roll mill.

25 A magnetic paste 213 included in a coating layer 13 is provided so as to cover the burned-out portion 41 and the coil conductor composition 221. The magnetic paste 213 is not particularly limited, and is prepared by, for example, screen-printing a first magnetic paste shown below.

30 The first magnetic paste is a paste composition, and can be formed by, for example, kneading a solvent, a raw material powder 132 that is prepared by calcining a magnetic ferrite material 131, a resin, and a plasticizer with a planetary mixer, and then dispersing the mixture with a three-roll mill. Examples of the solvent include a ketone-based solvent, examples of the resin include polyvinyl 35 acetal, and examples of the plasticizer include an alkyd-based plasticizer. As the magnetic ferrite material 131 and the raw material powder 132, the same materials as the magnetic ferrite material 111 and the raw material powder 112 can be used.

35 Then, a second magnetic composition 212 included in the second magnetic layer 12 is provided on the first magnetic sheet 211 in the same layer as the coil conductor composition 221. The second magnetic composition 212 can be formed by screen-printing a second magnetic paste 40 described below.

45 The second magnetic paste is a paste composition, contains a solvent, a raw material powder 122, a resin, and a

plasticizer, and can be formed by kneading these components with a planetary mixer, and then dispersing the mixture with a three-roll mill.

The raw material powder 122 can be prepared by calcining a magnetic ferrite material 121. As the magnetic ferrite material 121, the same material as the magnetic ferrite material 111 is used. The calcined magnetic ferrite material 121 can be prepared by wet-mixing and wet-grinding in which an ordinary method is used, and then drying the resulting product, and calcining the resulting dried product at 800° C. or more and 820° C. or less (i.e., from 800° C. to 820° C.). Note that there is a possibility that the raw material powder 122 will contain an inevitable impurity.

The coil conductor layer 21 is formed on the first magnetic layer 11 by the method shown in FIGS. 5A to 5E described above.

As shown in FIG. 6A, the extended conductor layer 61 is formed by, first, preparing the first magnetic sheet 211, and then, as shown in FIG. 6B, screen-printing a second conductor paste 261 on the first magnetic sheet 211. The extended conductor layer 62 is also formed in the same manner as the extended conductor layer 61.

The second conductor paste 261 is a paste composition, contains 100 parts by weight of an Ag powder and 0.2 parts by weight or more and 1.0 part by weight or less (i.e., from 0.2 parts by weight to 1.0 part by weight) of a ceramic powder such as  $\text{Al}_2\text{O}_3$  or  $\text{ZrO}_2$ , and is formed by dispersing these components.  $\text{Al}_2\text{O}_3$  and  $\text{ZrO}_2$  suppress the sintering of Ag during firing. Therefore, when  $\text{Al}_2\text{O}_3$  and  $\text{ZrO}_2$  are contained, the growth of an Ag grain can be suppressed. As a result, the average crystal grain size of the extended conductor layer 61 can be less than that of the coil conductor layer 21.

A laminate block is prepared by thermal pressure bonding of the above-described constituents. At this time, the pore area rate of the first magnetic layer 11 corresponding to the vicinity area E can be reduced by the thermal pressure bonding.

Then, the formed laminate block is subjected to an ordinary operation such as separation, firing, or formation of an external electrode to form a coil component 1. The separation, the firing, and the formation of an external electrode can be performed using an ordinary method. For example, the separation can be performed by cutting the obtained laminate block with a dicer or the like. If necessary, a rotary barrel is used to round the corner and the like. The firing can be performed at a temperature of 880° C. or more and 920° C. or less (i.e., from 880° C. to 920° C.). The formation of an external electrode can be performed by immersing the end face with the exposed extended conductor layer in a layer in which an Ag paste is extended to a predetermined thickness, baking the end face at a temperature of about 800° C. to form a base electrode, and then forming a Ni film and a Sn film in order on the base electrode by electrolytic plating.

By forming the coil component 1 as described above, the pore area rate in the non-vicinity area F is more than the pore area rate in the vicinity area E. Specifically, by the forming as described above, the pore area rate in the non-vicinity area F was 2.9%, the pore area rate in the vicinity area was 0.4% in each of the vicinity areas located above and below the coil conductor layer, and 0.3 to 0.6% in the vicinity areas located on the left and the right of the coil conductor layer.

The reason why the pore area rate has such a relationship is considered as follows. The raw material powder 122 contained in the second magnetic paste used for forming the second magnetic layer 12 is formed at a higher calcination

temperature than the raw material powder 112 used for forming the first magnetic layer 11. As a result, the density of the second magnetic layer 12 is relatively lower than the density of the first magnetic layer 11. That is, the pores included in the second magnetic layer 12 increases, and the pore area rate in the second magnetic layer 12 is more than the pore area rate in the first magnetic layer 11.

## Second Embodiment

FIG. 7 is an enlarged sectional view showing a coil conductor layer 21 included in a coil component 1 in a second embodiment and a void 51 provided on the lower face of the coil conductor layer 21. In the present embodiment, the coil conductor layer 21 has an elliptical shape. In the second embodiment, the configuration is the same as that of the coil component 1 in the first embodiment, except that the coil conductor layer 21 has the shape shown in FIG. 7. Descriptions of the same configuration as that in the first embodiment will be omitted.

What is claimed is:

1. A coil component comprising:  
an element body; and  
a coil provided in the element body and spirally wound  
along a first direction,  
the coil having a plurality of coil conductor layers stacked  
along the first direction,  
the element body having a vicinity area located in a  
vicinity of each of the coil conductor layers and having  
a non-vicinity area other than the vicinity area,  
the vicinity area having a pore area rate less than a pore  
area rate in at least a portion of the non-vicinity area,  
the vicinity area surrounds each of the coil conductor  
layers when viewed in a section view orthogonal to a  
length direction of each of the coil conductor layers,  
and  
the vicinity area is provided within 20  $\mu\text{m}$  from a surface  
of each of the coil conductor layers.
2. The coil component according to claim 1, wherein  
the element body has a first magnetic layer and a second  
magnetic layer,  
the first magnetic layer and the second magnetic layer are  
alternately stacked along the first direction, and  
the second magnetic layer is provided on the first mag-  
netic layer and exists in a same layer as each of the coil  
conductor layers.
3. The coil component according to claim 1, wherein  
the pore area rate in the vicinity area is 1% or less.
4. The coil component according to claim 1, wherein  
the pore area rate in at least a portion of the non-vicinity  
area is from 2% to 8%.
5. The coil component according to claim 1, wherein  
a difference between the pore area rate in the vicinity area  
and the pore area rate in at least a portion of the  
non-vicinity area is 1% or greater.
6. The coil component according to claim 1, wherein  
the element body further includes a void, and  
the void is located between the coil conductor layers  
adjacent to each other along the first direction, and is in  
contact with one coil conductor layer of the coil con-  
ductor layers adjacent to each other.
7. The coil component according to claim 2, wherein  
the pore area rate in the vicinity area is 1% or less.
8. The coil component according to claim 2, wherein  
the pore area rate in at least a portion of the non-vicinity  
area is from 2% to 8%.

**11**

9. The coil component according to claim 3, wherein the pore area rate in at least a portion of the non-vicinity area is from 2% to 8%.
10. The coil component according to claim 7, wherein the pore area rate in at least a portion of the non-vicinity area is from 2% to 8%.
11. The coil component according to claim 2, wherein a difference between the pore area rate in the vicinity area and the pore area rate in at least a portion of the non-vicinity area is 1% or greater. 10
12. The coil component according to claim 3, wherein a difference between the pore area rate in the vicinity area and the pore area rate in at least a portion of the non-vicinity area is 1% or greater. 15
13. The coil component according to claim 4, wherein a difference between the pore area rate in the vicinity area and the pore area rate in at least a portion of the non-vicinity area is 1% or greater.
14. The coil component according to claim 7, wherein a difference between the pore area rate in the vicinity area and the pore area rate in at least a portion of the non-vicinity area is 1% or greater. 20
15. The coil component according to claim 8, wherein a difference between the pore area rate in the vicinity area and the pore area rate in at least a portion of the non-vicinity area is 1% or greater. 25

**12**

16. The coil component according to claim 9, wherein a difference between the pore area rate in the vicinity area and the pore area rate in at least a portion of the non-vicinity area is 1% or greater.
17. The coil component according to claim 2, wherein the element body further includes a void, and the void is located between the coil conductor layers adjacent to each other along the first direction, and is in contact with one coil conductor layer of the coil conductor layers adjacent to each other.
18. The coil component according to claim 3, wherein the element body further includes a void, and the void is located between the coil conductor layers adjacent to each other along the first direction, and is in contact with one coil conductor layer of the coil conductor layers adjacent to each other.
19. The coil component according to claim 4, wherein the element body further includes a void, and the void is located between the coil conductor layers adjacent to each other along the first direction, and is in contact with one coil conductor layer of the coil conductor layers adjacent to each other.
20. The coil component according to claim 5, wherein the element body further includes a void, and the void is located between the coil conductor layers adjacent to each other along the first direction, and is in contact with one coil conductor layer of the coil conductor layers adjacent to each other.

\* \* \* \* \*